# EUROPEAN PATENT SPECIFICATION

(11) **EP 0 154 548 B1**
(45) Date of publication and mention of the grant of the patent: **30.08.1989**
(21) Application number: 85301507.1
(22) Date of filing: 05.03.1985
(51) Int. Cl.: B22F 9/30, C22C 1/04, B22F 3/00

(54) **Amorphous metal alloy powders and bulk objects and synthesis of same by solid state decomposition reactions**
Pulver und Körper aus amorphen Metallegierungen und ihre Synthese in fester Phase durch Zersetzungsreaktionen
Poudres et objets massifs en alliage métallique amorphe et leur synthèse par réaction de décomposition en phase solide

(30) Priority: 05.03.1984 US 586380; 05.03.1984 US 586467
(43) Date of publication of application: 11.09.1985
(73) Proprietor: THE STANDARD OIL COMPANY, Cleveland, Ohio 44115 (US)
(72) Inventor: Tenhover, Michael Alan, Solon Ohio 44139 (US); Grasselli, Robert Karl, Aurora Ohio 44202 (US); Henderson, Richard Scott, Solon Ohio 44139 (US)
(74) Representative: Smith, Sydney

(56) References cited:
- WO-A-84/02926
- DE-A- 3 014 121
- US-A- 2 686 714
- US-A- 4 282 034
- MACHINE DESIGN, vol. 55, no. 25, 10th November 1983, page 8, Penton/IPC, US; "New method for making amorphous metals"
- PHYSICAL REVIEW LETTERS, vol. 51, no. 5, 1st August 1983, pages 415-418, California Institute of Technology, Pasadena, Ca., US; R.B. SCHWARZ et al.: "Formation of an amorphous alloy by solid-state reaction of the pure polycrystylline metals"

## Description

### Field of the invention

This invention relates to amorphous metal alloy powders and shapes and the novel preparation of such powders by solid state reactions. More specifically, this invention relates to the synthesis of amorphous metal alloy powders by the thermal decomposition of metal-bearing compounds and the synthesis of amorphous metal alloy shapes by solid state reactions that utilize a ductile matrix precursor.

### Background of the invention

Amorphous metal alloy materials have become of interest in recent years due to their unique combinations of mechanical, chemical and electrical properties that are especially well-suited for newly-emerging applications. Examples of amorphous metal material properties include the following:
-uniform electronic structure,
-compositionally variable properties,
-high hardness and strength,
-flexibility,
-soft magnetic and ferroelectronic properties,
-very high resistance to corrosion and wear,
-unusual alloy compositions, and
-high resistance to radiation damage.

These characteristics are desirable for applications such as low temperature welding alloys, magnetic bubble memories, high field superconducting devices and soft magnetic materials for power transformer cores.

The unique combination of properties of amorphous metal alloy materials may be attributed to the disordered atomic structure of amorphous materials which ensures that the material is chemically homogeneous and free from the extended defects, such as dislocations and grain boundaries, that are known to limit the performance of crystalline materials. The amorphous state is characterized by a lack of long range periodicity, whereas a characteristic of the crystalline state is its long range periodicity.

Generally, the room temperature stability of amorphous materials depends on various kinetic barriers to the growth of crystal nuclei and to nucleation barriers that hinder the formation of stable crystal nuclei. Such barriers typically are present if the material to be made amorphous is first heated to a molten state then rapidly quenched or cooled through the crystal nucleation temperature range at a rate that is sufficiently fast to prevent significant nucleation to occur. Such cooling rates are on the order of 10⁶°CI second. Rapid cooling dramatically increases the viscosity of the molten alloy and quickly decreases the length over which atoms can diffuse. This has the effect of preventing crystalline nuclei from forming and yields a metastable, or amorphous phase.

Processes that provide such cooling rates include sputtering, vacuum evaporation, plasma spraying and direct quenching from the liquid state. It has been found that alloys produced by one method often cannot be similarly produced by another method even though the pathway to formation is in theory the same.

Direct quenching from the liquid state has found the greatest commercial success since a variety of alloys are known that can be manufactured by this technique in various forms such as thin films, ribbons and wires. United States patent number 3,856,513 to Chen et al. describes novel metal alloy compositions obtained by direct quenching from the melt and includes a general discussion of this process. Chen et al. describes magnetic amorphous metal alloys formed by subjecting the alloy composition to rapid cooling from a temperature above its melting temperature. A stream of the molten metal is directed into the nip of rotating double rolls maintained at room temperature. The quenched metal, obtained in the form of a ribbon, was substantially amorphous as indicated by x-ray diffraction measurements, was ductile, and had a tensile strength of about 350,000 psi (2,413,250 kPa).

United States patent number 4,036,638 to Ray et al. describes binary amorphous alloys of iron or cobalt and boron. The claimed amorphous alloys were formed by a vacuum melt-casting process wherein molten alloy was ejected through an orifice and against a rotating cylinder in a partial vacuum of about 100 millitorr 13.332 Pa. Such amorphous alloys were obtained as continuous ribbons and all exhibited high mechanical hardness and ductility.

The thicknesses of essentially all amorphous foils and ribbons formed by rapid cooling from the melt are limited by the rate of heat transfer through the material. Generally the thicknesses of such films are less than 50 pm. The few materials that can be prepared in this manner include those disclosed by Chen et al. and Ray et al.

Amorphous metal alloy materials prepared by electrodeposition processes have been reported by Lashmore and Weinroth in Plating and Surface Finishing, 72 (August 1982). These materials include Co-P, Ni-P, Co-Re and Co-W compositions. However, the as-formed alloys are inhomogeneous and so can be used in only a limited number of applications.

The above-listed prior art processes for producing amorphous metal alloys depend upon controlling the kinetics of the solidification process; controlling the formation of the alloy from the liquid (molten) state or from the vapor state by rapidly removing heat energy during solidification. Most recently, an amorphous metal alloy composition was synthesized without resort to rapid heat removal. Yeh et al. reported that a metastable crystalline compound Zr₃Rh, in the form of a thin-film could be transformed into a thin-film, amorphous metal alloy by the controlled introduction of hydrogen gas; Applied Physics Letter 42 (3), pp. 242-244, February 1, 1983. The amorphous metal alloy had an approximate composition of Zr₃RhH₅.₅.

Yeh et al. specified three requirements as prerequisites for the formation of amorphous alloys by solid state r reactions: at least a three component system; a large disparity in the atomic diffusion rates of two of the atomic species; and an absence of a polymorphic crystalline alternative as a final state. Thus, Yeh et al. teach that solid state reactions would have limited applications for the synthesis of amorphous metal alloy materials.

The known amorphous metal alloy and processes for making such alloys which are discussed above suffer from the disadvantage that the so-formed amorphous alloy is produced in a limited form, that is, as a thin film such as a ribbon, wire or platelet. These limited shapes place severe restrictions on the applications for which amorphous metal materials may be used.

To produce bulk amorphous metal alloy objects the formed amorphous alloy must be mechanically reduced to a powder as by chipping, crushing, grinding and ball milling, and then re-combined in the desired shape. These are difficult processes when it is realized that most amorphous metal alloys have high mechanical strengths and also possesses high hardnesses.

In Amorphous Metallic Alloys, F. E. Luborsky, 1983, pages 506-521 there is described the production of certain amorphous powders, for example C_{U6o}Zr₄ₒ, by using ultrasonic gas atomization. XRD analysis of amorphous Cu₆ₒZr₄ₒ powder prepared using helium gas indicates particle sizes below 50 pm to be fully amorphous and to have increasing crystalline content as the size approaches 125 pm.

What is lacking in the area of amorphous metal alloy preparation is a simple process for the direct formation of a large variety of amorphous metal alloys. Especially lacking is a process that would synthesize amorphous metal alloy materials directly as powders suitable for forming bulk amorphous metal alloy shapes.

Hence, it is one object of the present invention to provide novel amorphous metal alloy compositions.

It is another object of the present invention to provide a process for the direct preparation of a large variety of homogeneous amorphous metal alloy compositions.

It is a further object of the present invention to provide a process for the direct preparation of a large variety of homogeneous amorphous metal alloy compositions in a powder form.

It is still another object of the present invention to provide a process for the direct preparation of a large variety of homogeneous amorphous metal alloy powders by solid state reaction.

It is yet another object of this invention to provide novel bulk amorphous metal alloy objects.

It is another object of the present invention to provide a process for the synthesis of bulk amorphous metal alloy objects.

These and additional objects of the present invention will become apparent in the description of the invention and examples that follow.

### Summary of the invention

The present invention relates to a process for the synthesis of an at least 50% amorphous metal alloy comprising thermally decomposing at least one precursor metal-bearing compound selected from organometallic compounds such as monomers, dimers, trimers and polymers having metallo-organic ligands composed of saturated and/or unsaturated hydrocarbons, aromatic or heteroaromatic ligands, or oxygen, boron, carbon, nitrogen, phosphorus, arsenic, germanium, antimony and/or silicon containing ligands; halogen compounds; oxides; nitrates; nitrides; carbides; carbonyls, borides or metal-bearing salts, at a temperature below the crystallization temperature of the amorphous metal alloy to be formed, the at least one precursor metal-bearing compound having a decomposition temperature below the crystallization temperature of the amorphous alloy to be formed to form a decomposition product of the following empirical formulae:-
wherein M is at least one metal selected from the metals in Groups VI-A, VII-A, VIII, IA, IIA and IIIA of the Periodic Table; and
X is at least one element selected from Groups III-B, IV-B and V-B of the Periodic Table; and
wherein a ranges from about 0.1 to about 0.9; and
wherein N is at least one metal selected from the metals in Groups III-A, IV-A, V-A and VI-A of the Periodic Table; and
Y is selected from Groups VIII, I-A and II-A of the Periodic Table; and
wherein b ranges from about 0.2 to about 0.8 and containing the metals which comprise the amorphous metal alloy to form the desired amorphous metal alloy or to form an intimate mixture of the components of the amorphous metal alloy which is then heat treated at a temperature below the crystallization temperature of the amorphous metal alloy to be formed to form the amorphous metal alloy.

The amorphous metal alloy is at least fifty percent amorphous. Preferably the metal alloy is at least eighty percent amorphous and most preferably about one hundred percent amorphous, as indicated by x-ray diffraction analysis. The use of the phrase "amorphous metal alloys" herein refers to amorphous metal-containing alloys that may also comprise non-metallic elements. Amorphous metal alloys may include non-metallic elements such as boron, carbon, nitrogen, silicon, phosphorus, arsenic, germanium and antimony.

The solid state processes disclosed herein include the step of thermally decomposing the at least one precursor metal-bearing compound at a temperature below the crystallization temperature of the amorphous metal alloy to be formed. The at least one precursor metal-bearing compound is preferably chosen so that its decomposition temperature is at least 25°C below the crystallization temperature of the amorphous metal alloy to be formed and most preferably is at least 100°C below the crystallization temperature of the armosphous metal alloy to be formed.

Typical precursor metal-bearing compounds have decomposition temperatures between about 20°C and about 500°C. A substantial number of precursor metal-bearing compounds suitable for use in the processes of this invention have decomposition temperatures between about 150°C and about 400°C.

The thermal decomposition of the at least one precursor metal-bearing compound yields an intimate mixture of the components of the desired metal alloy. This decomposition step is preferably performed in a reactor having collection means so that about a one hundred percent yield of material will be realized. This may be achieved by maintaining a cooled reactor portion downstream of the thermal decomposition portion of the reactor wherein the thermally decomposed products will be deposited. Alternatively and most preferably, the decomposition step may be performed in a sealed reactor to prevent evaporation of the metal alloy components. Upon cooling, about a one hundred percent yield of the reaction products may be recovered therefrom.

The decomposition of the precursor compounds may occur under an atmosphere suitable for the synthesis of the desired amorphous metal alloy. The precursor compounds may be disposed in a sealed reaction vessel that has been partially or fully evacuated prior to heating. If the amorphous metal alloy to be synthesized does not contain oxygen, then it is preferred that the thermal decomposition of the precursor compounds be done under an inert or reducing atmosphere or in a sealed reaction vessel that has been partially or fully evacuated. If some tolerance to oxygen is possible then an inert or reducing atmosphere or vacuum may not be necessary.

A precursor compound may also exist at room temperature in the gaseous state and may itself provide the initial atmosphere under which the thermal decomposition will be performed. In this manner, a reactive atmosphere exists for the thermal decomposition reaction. Precursor compounds may also be used that are solid at about 20°C, but which vaporize at slightly elevated temperatures. These compounds may be disposed in an evacuated reactor and upon heating, provide a reactive atmosphere for the decomposition reaction.

The precursor metal-bearing compounds suitable for use in this invention are organometallic compounds such as monomers, dimers, trimers and polymers having metallo-organic ligands composed of saturated and/or unsaturated hydrocarbons, aromatic or heteroaromatic ligands, and may also include oxygen, boron, carbon, nitrogen, phosphorus, arsenic, germanium, antimony and/or silicon-containing ligands, and combinations thereof. Precursor metal-bearing compounds may also be halogen compounds, oxides, nitrates, nitrides, carbides, carbonyls, borides or metal-bearing salts, with the restriction that the decomposition temperature of the precursor compound be less than the crystallization temperature of the amorphous metal alloy to be synthesized.

As disclosed earlier, precursor compounds may also be provided that do not contain a metal but which contribute a non-metallic element to the amorphous alloy composition.

The thermal decomposition of precursor compounds yields a product consisting essentially of the components of the desired amorphous metal alloy. The components are intimately mixed, the maximum size of the particles in the mixture preferably being from about 10 Angstroms to about 1000 Angstroms, (10⁻¹⁰―1,000⁻¹⁰ m) and most preferably from about 10 Angstroms to about 500 Angstroms (10-'⁰⁻500-¹⁰ m).

The thermal decomposition of the precursor compounds may occur at high enough temperatures and for a period of time long enough to permit alloying of the metal elements concurrent with the decomposition. Under such circumstances the product which results from the decomposition step is a substantially amorphous metal alloy.

This product is synthesized as a solid, powder material having a maximum particle size of from about 10 Angstroms (10xlO-" m) to about 1000 Angstroms (1,000x10⁻¹⁰ m). This powder is suitable for compaction, with or without a binder, into a solid shape.

If the decomposition temperature is not sufficiently high, or the period of decomposition is too brief, to enable alloying of the reactant products during the decomposition of the precursor compounds, then the powder that is obtained is an intimate mixture comprising the alloy components. A subsequent heat-treating step at a temperature below the crystallization temperature of the amorphous metal alloy will allow diffusion of at least one metal component so as to form an amorphous metal alloy. This heat-treating step is carried out under an atmosphere conducive to the formation of the amorphous metal alloy. This may occur under vacuum conditions, from about 0 torr to about 500 torr (66,500 Pa) or in an inert, reducing or reactive atmosphere.

Prior to the heat-treating step, the powder obtained from the decomposition of the precursor compounds may be pressed into a shape so that, upon heat-treating, a bulk amorphous metal alloy shape is obtained. It is also possible to compact the heat-treated amorphous metal alloy powder into a solid shape.

It has also surprisingly been found that the amorphous metal alloy products of thermal decomposition and decomposition/heat-treating processes may be mixed with another precursor metal-bearing compound to yield a new, enhanced amorphous metal alloy material which has incorporated into the prior amorphous metal alloy elements from the newly-added precursor. This may be accomplished by disposing the prior amorphous metal alloy in a reactor with the newly-added precursor metal-bearing compound and heat-treating this mixture at a temperature that will decompose the precursor compound but that is below the crystallization temperatures of the prior amorphous metal alloy and the enhanced amorphous metal alloy that is to be synthesized. The newly-added precursor may be a solid, liquid or gaseous material upon insertion into the reaction vessel. As with the above- discussion, the decomposition of the precursor material may occur in a partial or full vacuum, or under an inert, reducing, or reactive atmosphere.

The solid state reaction that occurs to alloy an intimate mixture of elements may be viewed by examining the free energy of the system. The intimate mixture of elements corresponds to a relatively high free energy of the system. At about room temperature such mixtures are generally kinetically restricted to this state. Adding energy to this system, as at the thermal decomposition temperature or during subsequent heat-treatments, allows the componnets to begin to inter- diffuse. The free energy of the system is lowered by an increase in the entropy of mixing a decrease in the enthalpy due to the formation of heteropo- lar bonds. The absolute minimum in free energy in these systems will occur for the equilibrium crystalline alloys. For many alloy combinations, however, a local minimum in the free energy can exist in an amorphous phase. For alloy combinations such as these, the requirements for the formation of an amorphous phase by a solid state reaction are that the intimate mixture of components have a free energy higher than that of the amorphous phase and that the diffusion process to form the alloy be performed at temperatures sufficiently below the characteristic temperatures for the formation of crystalline nuclei.

Amorphous metal alloys are generally characterized as having high strengths and hardnesses and so are quite resistant to deformation. Typical amorphous shapes, such as ribbons and wires, are formed simultaneously with the formation of the amorphous state. These shapes exhibit the characteristics of an amorphous material. However, attempts to form bulk amorphous shapes, that is, shapes having significant thicknesses in all dimensions, have not been satisfactory. These attempts generally include reducing an amorphous metal alloy, such as a ribbon, to an amorphous powder by physical means and then compacting the powder into a shape. Generally, the compacted shape does not retain all the desirable traits of the individual particles.

Whereas the process disclosed herein above teaches the synthesis of amorphous metal alloy powders, it now becomes known, in accordance with the invention claimed herein, that the intimate mixture obtained as an intermediate in the formation of Applicants' amorphous metal alloy powders may be effectively formed into bulk objects when at least one component of the intimate mixture is ductile. By ductile is meant a component that is malable, pliant and easily molded without cracking or fracturing. A typical ductile component will demonstrate deformation of at least ten percent under a moderate load of between about 1,000 psi (6895 kPa) and 5,000/psi (34,475 kPa). The ductile component of the intimate mixture provides an infrastructure that, when subjected to forming processes, deforms and binds the other components of the alloy within a matrix.

The ductile component of the alloy originates in a precursor compound that is used in the solid state reactions to form the intimate mixture of the alloy components. Examples of ductile components include pure metal elements, such as iron, nickel, copper, cobalt and tantalum, and metal solid solutions.

To provide enhanced bonding strength and properties to the formed amorphous metal alloy object, it is preferred that the ductile component comprise from about 10 atomic percent to about 95 atomic percent of the amorphous metal alloy based on the total composition of the amorphous metal alloy.

The intimate mixture of the components of the amorphous metal alloy, which has not yet been heat-treated to induce the amorphous state is subjected to a forming process. Forming processes include well-known powder forming techniques such as cold-pressing, hot-pressing, pressureless sintering, slipcasting, injection molding and extrusion. In accordance with this invention, the only restriction on the forming process is that the process be performed at a temperature below the crystallization temperature of the metal alloy.

If the forming process includes the use of temperature above ambient temperature, then the intimate mixture may be formed and made amorphous simultaneously. If the forming process does not include elevated temperatures, then a further step, heat-treating, will be required to induce the amorphous state.

Many intimate mixtures may be reactive with oxygen, and so, may require forming and heat-treating processing which occurs in an oxygen- free atmosphere such as an inert, reducing or reactive atmosphere or under vacuum conidtions. A reactive atmosphere may be provided that reacts with the bulk object so as to enhance the formation of the amorphous alloy.

Amorphous metal alloy shapes generally have a density of from about 10 percent to about 99 percent of theoretical. The density may be controlled by the forming process so as to meet a variety of needs. Thus, the same amorphous metal alloy composition may be formed into an amorphous metal alloy shape having a density between about 10 percent and about 90 percent of theoretical. It has also been observed that the process of this invention permits the attainment of a desired-density object at temperatures lower than those necessary to achieve the same sintered state when the metal alloy powder used to form the object is derived from the physical reduction of a prior art, thin-film amorphous shape such as a ribbon.

The forming process may be used to provide an amorphous metal alloy in a finished shape or in a solid shape amenable to further machining. Thus, billits, rods, flatplates may be formed as well as cylindrical shapes, toroids and other intricate, finished shapes.

The above-described processes for synthesizing amorphous metal alloys are not hindered by the processing limitations of prior art processes. The methods disclosed herein do not depend on extremely high cooling rates or heat transfer properties, nor is very high temperature or very low vacuum equipment necessary. Further, the processes of this invention provide for the synthesis of substantially amorphous metal alloy powders, which amorphous alloy powders may be pressed into desired shapes to form solid amorphous alloy shapes. Alternatively, the methods disclosed herein provide an intimate mixture of elements that may be formed into a desired shape and, upon subsequent heat-treating, may be converted into a substantially amorphous metal alloy shape. The method disclosed herein does not depend on reducing an amorphous material to a powder state and then recombining an amorphous powder but utilizes an intimate mixture of the components of a metal alloy into a bulk shape and thereafter, or concurrently, inducing the amorphous state by heat treating at a temperature below the crystallization temperature of the metal alloy. These bulk amorphous metal alloy shapes may find new and useful applications, since such shapes have not been conveniently fabricated by any other techniques.

### Examples

The following examples more thoroughly illustrate the present invention and are not intended in any way to be limitative thereof. Each of the following examples describes the co-decomposition of organometallic compounds to yield amorphous metal alloy powders.

### Example 1

This example demonstrates the formation of an amorphous iron-molybdenum composition.

Equimolar amounts of about 2 mmol each of cyclopentadienyliron dicarbonyl dimer [C_{S}H_{S}Fe(CO)₂]₂ and cyclopentadienylmolybdenum tricarbonyl dimer [C₅H₅M_{O}(CO₃)1₂ were disposed in a stainless steel bomb reactor. The reactor was purged with argon and sealed under an argon atmosphere. The bomb reactor was then heated to a temperature of about 300°C for about 24 hours. The decomposition temperature of cyclopentadienyliron dicarbonyl dimer is about 195°C, and the decomposition temperature of cyclopentadienylmolybdenum tricarbonyl dimer is about 180°C.

After cooling to about 20°C, the reactor was opened and a black-colored solid, in powder form, was removed therefrom. The powder was washed with tetrahydrofuran to remove any organic-soluble materials, then dried at a temperature of about 60°C under vacuum.

The powder was next divided into four fractions, a first fraction was set aside for later analysis, and the other three fractions were further treated in the following manner: one fraction was heat-treated at about 270°C under vacuum for about 168 hours, another fraction was heat-treated about 325°C under vacuum for about 168 hours, and still another fraction was heat-treated at about 800°C under vacuum for about 10 minutes.

X-ray diffraction data indicated that the powder removed from the bomb reactor after co-decomposition of the precursor materials comprised an amorphous iron-molybdenum alloy having an approximate composition of Fe₅₀Mo₅₀(Fe_{0.5}Mo_{0.5}). The fractions of the powder that were heat-treated at about 270°C and about 325°C were also found to comprise an amorphous iron-molybdenum alloy of approximate composition FesoMo₅o (Feo.5Moo.5), as indicated by x-ray diffraction, but the fraction of the powder that was heat-treated at about 800°C was crystalline.

Differential scanning calorimetry was implemented to determine that the atmosphous alloy powder fractions had glass transition temperatures of about 325°C and crystallization temperatures of about 420°C. Mossbauer Effect Spectra of the amorphous powder fractions indicated that these amorphous iron-molybdenum alloy powders have internal magnetic fields and magnetic moments similar to other iron-containing amorphous alloys.

Amorphous iron-molybdenum alloy compositions have not been reported as formed by any other method except sputtering, which method cannot synthesize the amorphous alloy in powder form.

### Example 2

This example demonstrates the formation of an amorphous iron-molybdenum composition using alternative precursor organometallic compounds.

Equimolar amounts of iron pentacarbonyl (Fe(CO)₅) and molybdenum carbonyl (Mo(CO)₆) could be sealed under an inert atmosphere such as an argon atmosphere or under a vacuum in a bomb reactor and heated to about 270°C for about 120 hours to thermally decompose about all of the precursor compounds and to alloy the reactant product elements. The decomposition temperature of iron pentacarbonyl is about 150°C, and the decomposition temperature of molybdenum carbonyl is about 150°C.

The resultant solid, powder material that is obtained by this decomposition can be confirmed by x-ray diffraction to be amorphous iron-molybdenum alloy. The approximate composition will be amorphous Fe₅ₒMo₅ₒ (Feo.₅Moo.₅).

### Example 3

This example demonstrates the formation of an amorphous iron-molybdenum nitrogen composition.

Equimolar amounts of iron pentacarbonyl (Fe(CO)₅) and molybdenum carbonyl (Mo(CO)₆) may be disposed in a reactor and sealed under an atmosphere of ammonia. The reactor could then be heated to a temperature above the decomposition temperatures of iron pentacarbonyl and molybdenum carbonyl, which is above about 270°C for a period of time that would insure decomposition of the reactant materials and alloying of the component elements.

The product that would be obtained as a solid powder material will be an amorphous iron-molybdenum-nitrogen alloy of approximate composition Fe₄₀Mo₄₀N₂₀ (Fe_{0.4}Mo_{0.4}N_{0.2}), the nitrogen having been derived from the ammonia atmosphere under which the solid products were sealed prior to heating.

### Example 4

This example describes the formation of an amorphous iron-chromium-molybdenum composition.

The following three organometallic precursor materials could be disposed in a bomb reactor in about the following molar ratios: 1.0 mol equivalent iron dodecarbonyl (Fe₃(CO)₁₂), 0.5 mol equivalent chromium carbonyl (Cr(CO)₆), and 3 mol equivalents molybdenum carbonyl (Mo(CO)s). The decomposition temperature of iron dodecarbonyl is about 140°C. The decomposition temperature of chromium carbonyl is about 200°C. The decomposition temperature of molybdenum carbonyl is about 150°C.

The reactor may then be sealed under an inert atmosphere and heated to a temperature above about 270°C for a period of time sufficient to decompose the precursor compounds and to alloy the elements of the amorphous composition.

The solid, powder material that is obtained from this thermal decomposition will be an amorphous iron-chromium-molybdenum material of approximate composition Fe₃Crₒ.₅Mo₃ (Fe_{0.46}Cr_{0.08}^{MO}_{0.46}).

### Example 5

Example 4 above could also have been performed under an atmosphere other than an inert atmosphere so as to modify the product amorphous metal alloy.

The inert atmosphere of Example 4 may be replaced with a phosphorus atmosphere obtained by disposing solid elemental phosphorus, such as red phosphorus, in the reactor with the other precursor compounds and sealing the reactor under a vacuum. At elevated temperatures, the phosphorus would vaporize producing a phosphorus atmosphere during the decomposition of the other precursor compounds. The resultant amorphous metal alloy from the thermal decomposition reaction may have an approximate composition of PFe₃Crₒ.ₛMO₃ (P_{0.3}Fe_{0.4}Cr_{0.07},Mo_{0.4}).

### Example 6

This example demonstrates the formation of an amorphous tungsten-nickel-carbon composition.

Precursor materials, mesitylene tungsten tricarbonyl (C₉H₁₂W(CO)₃) and bis(triphenylphosphine) nickel dicarbonyl ((C₆H₅)₃P]₂Ni(CO)₂, may be disposed in a bomb reactor in a molar ratio of about 1:2. The decomposition temperature of mesitylene tungsten tricarbonyl is about 165°C, and the decomposition temperature of bis(triphenylphosphine) nickel dicarbonyl is about 215°C. The reactor may be sealed under an inert atmosphere such as an argon atmosphere and then heated to a temperature above about 215°C for a time long enough to insure that the precursor compounds have substantially decomposed and alloyed.

A solid, powder material would result that is an amorphous tungsten-nickel-carbon-phosphorus material having an approximate composition of WNi₂Cₒ.ₛP (W_{0.22}Ni_{0.44}C_{0.12}P_{0.22}).

### Example 7

The formation of an amorphous cobalt rhenium composition is described in this example.

The following two organometallic precursor materials may be disposed in a bomb reactor in about the following molar ratios: 1 mol rhenium carbonyl (Re₂(CO)₁₀) and 2 mols cobalt carbonyl (C0₂(CO)ₛ). The reactor may then be sealed under an inert atmosphere, such as an argon atmosphere and heated to about at least 170°C for a time sufficient to thermally decompose the precursor compounds. The decomposition temperature of rhenium carbonyl is about 170°C. The decomposition temperature of cobalt carbonyl is about 55°C. The resultant solid, powder material that is obtained by this decomposition will be an amorphous alloy of cobalt rhenium. The approximate composition will be amorphous Co₂Re (Co_{0.67}Re_{0.33}).

### Example 8

The formation of an amorphous tungsten- cobalt-iron composition is described in this example.

The following organometallic precursor materials may be disposed in a bomb reactor in about the following molar ratios: 1 mol equivalent tungsten carbonyl (W(CO)₆), 1 mol equivalent cobalt carbonyl (Co₂(CO)ₑ), and 2 mols equivalents iron noncarbonyl (Fe₂(CO)₉). Tungsten carbonyl has a decomposition temperature of about 170°C. Cobalt carbonyl has a decomposition temperature of about 55°C. Iron noncarbonyl has a decomposition temperature of about 100°C.

The reactor may be sealed under an inert amosphere and heated to a temperature above about 270°C so as to substantially thermally decompose the precursor compounds and to alloy the product elements.

The powder removed from the bomb reactor after the co-decomposition of the precursor materials will comprise an amorphous tungsten- cobalt-iron composition of approximately WCo₂Fe₄ (W_{0.14}CO_{0.28}Fe_{0.58}).

### Example 9

This example demonstrates the formation of an amorphous chromium-iron-nickel-boron composition synthesized by adding a chromium-bearing precursor compound to an amorphous iron-nickel-boron alloy.

Chromium carbonyl (Cr(CO)₆) was mixed with a substantially amorphous metal alloy of iron-nickel-boron, having an approximate composition Fe₂Ni₂B (Fe_{0.4}Ni_{0.4}B_{0.2}). in a molar ratio of about 1:2 and were then disposed in a bomb reactor, evacuated and sealed. Chromium carbonyl thermally decompose at about 200°C. The crystallization temperature of the amorphous Fe₂Ni₂B (Feₒ.₄Niₒ.₄Bₒ.₂) alloy is about 410°C, its glass transition temperature is about 330°C.

The sealed reactor was heated to about 250°C and maintained at about that temperature for about 120 hours. Upon cooling and opening the reactor and examining its components, no chromium carbonyl was found to be present. However, x-ray diffraction analysis determined that the powder that was removed from the reactor after this heat-treating was amorphous, having an approximate composition of Cro.ofe₂Ni₂B (G_{0.09}Fe_{o.36}Ni_{0.36}B_{0.1}). Thus, the process disclosed herein may include the enhancement of an amorphous metal alloy by further decomposing a metal-bearing precursor compound in the presence of an amorphous metal alloy whereby the metal in the precursor compound is incorporated into the alloy, and which alloy remains substantially amorphous.

The above-described examples demonstrate the formation of amorphous metal alloy compositions by decomposition of precursor metal-bearing materials. The formation of such amorphous materials could only be obtained previously by processes that utilize high temperature, energy intensive equipment. In addition, the novel processes described herein above produce amorphous metal alloy powders, whereas prior art processes yield the amorphous material only in a solid, thin-film or ribbon-like form which must first be reduced to a powder if it is to be formed into a solid shape.

This example demonstrates the formation of a solid shape having amorphous characteristics and an approximate composition of Fe₂Ni₂B (Fe_{0.4}Ni_{0.4}B_{0.2}).

### Example 10

In this Example, an intimate mixture of the components of the amorphous metal alloy was obtained by a chemical reduction process. Equimolar amounts of iron chloride, FeC12. 4H₂0, and nickel chloride, NiCI2. 6H₂0, were dissolved in distilled water to form a reaction solution. This solution was degassed with argon so as to purge oxygen from the solution. An argon-degassed solution of sodium borohydride, NaBH₄, was then added dropwise to the reaction solution. The solution was stirred for about sixteen hours to insure that the reaction had gone to completion.

A black precipitate was recovered from the solution and dried at about 60°C under vacuum. This precipitate was an intimate mixture of the components of the metal alloy to be formed. The intimate mixture comprised iron metal and nickel boride. The pure iron metal is the ductile component of the mixture.

This powder mixture was kept under an argon atmosphere to prevent oxidation and compacted into a disc having a diameter of about 1 cm and a thickness of about 0.1 cm at a pressure of about 10,000 psi (68,950 kPa) and at about 20°C. The disc was sealed in an evacuated glass tube and heat treated at about 250°C for about 312 hours.

X-ray diffraction analysis revealed that the resultant disc was a solid amorphous metal alloy having a composition of about Fe₂Ni₂B. This disc had a density that was about 98 percent of theoretical.

The formation of amorphous metal alloy shapes could only be formed previously by first reducing an already-amorphous material into a powder and then compacting the powder. Such a process is not desirable since it inherently is energy intensive and cannot reliably produce consistent, homogeneous amorphous shapes. The disadvantages of the prior art are removed with the above-described process.

## Claims

1. A process for the synthesis of an at least 50% amorphous metal alloy comprising thermally decomposing at least one precursor metal-bearing compound selected from organometallic compounds such as monomers, dimers, trimers and polymers having metallo-organic ligands composed of saturated and/or unsaturated hydrocarbons, aromatic or heteroaromatic ligands, or oxygen, boron, carbon, nitrogen, phosphorus, arsenic, germanium, antimony and/or silicon containing ligangs; halogen compounds; oxides; nitrates; nitrides; carbides; carbonyls; borides or metal-bearing salts at a temperature below the crystallization temperature of the amorphous metal alloy to be formed, the at least one precursor metal-bearing compound having a decomposition temperature below the crystallization temperature of the amorphous alloy to be formed to form a decomposition product of the following empirical formulae:-
wherein M is at least one metal selected from the metals in Groups VI-A, VII-A, VIII, IA, IIA and IIIA of the Periodic Table; and
X is at least one element selected from Groups III-B, IV-B and V-B of the Periodic Table; and
wherein a ranges from about 0.1 to about 0.9; and
wherein N is at least one metal selected from the metals in Groups III-A, IV-A, V-A and VI-A of the Periodic Table; and
Y is selected from Groups VIII, I-A and II-A of the Periodic Table; and
wherein b ranges from about 0.2 to about 0.8 and containing the metals which comprise the amorphous metal alloy to form the desired amorphous metal alloy or to form an intimate mixture of the components of the amorphous metal alloy which is then heat treated at a temperature below the crystallization temperature of the amorphous metal alloy to be formed to form the amorphous metal alloy.

2. A process as claimed in claim 1 characterised in that the substantially amorphous metal alloy is obtained as a powder.

3. A process as claimed in claim 2 characterised in that the powder is further processed into a solid shape.

4. A process as claimed in any of claims 1 to 3 characterised in that the intimate mixture of the components of the amorphous metal alloy to be synthesized is pressed into a shape.

5. A process as claimed in any of claims 1-4 characterised in that the thermal decomposition occurs under an inert atmosphere.

6. A process as claimed in any of claims 1 to 4 characterised in that the decomposition occurs under a reactive atmosphere.

7. A process as claimed in any of claims 1 to 6 characterised in that it synthesizes an amorphous metal alloy composition including nonmetallic elements.

8. A process as claimed in claim 7 characterised in that heat-treating of the intimate mixture occurs under an atmosphere comprising said nonmetallic elements.

9. A process as claimed in any of claims 1 to 8 characterised in that heat-treating of the intimate mixture is performed under an inert atmosphere.

10. A process as claimed in any of claims 1 to 9 characterised in that said heat-treating of the intimate mixture is performed under a reactive atmosphere.

11. A process as claimed in any of claims 1 to 10 characterised in that said intimate mixture comprises particles having a maximum particle size of from 10x10⁻¹⁰ m to about 1,00O_{X}10-¹⁰ m.

## Patentansprüche

1. Verfahren zur Synthese einer mindestens 50% amorphen Metallegierung, welches, umfaßt, die thermische Zersetzung von mindestens einer metallhaltigen Vorläuferbindung, ausgewählt aus organometallischen Verbindungen, wie Monomeren, Dimeren, Trimeren und Polymeren mit metallorganischen Liganden bestehend aus gesättigten und/oder ungesättigten Kohlenwasserstoffen, aromatischen oder heteroaromatischen Liganden, oder Sauerstoff, Bor, Kohlenstoff, Stickstoff, Phorphor, Arsen, Germanium, Antimon und/oder Silicium enthaltenden Liganden; Halogenverbindungen; Oxiden; Nitraten; Nitriden; Carbiden; Carbonylen; Boriden oder metallhaltigen Salzen, bei einer Temperatur unter der Kristallisationstemperatur der zu bildenden amorphen Metall-Legierung, wobei die mindestens eine metallhaltige Vorläuferverbindung eine Zersetzungstemperatur unter der Kirstallisationstemperatur der zu bildenden amorphen Legierung hat, unter Bildung eines Zersetzungsprodukts der folgenden empirischen Formeln:
worin M mindestens ein Metall ist, ausgewählt aus den Metallen der Gruppen VI-A, VII-A, VIII, IA, IIA und IIIA des Periodensystems; und
X mindestens ein Element ist, ausgewählt aus den Gruppen III-B, IV-B und V-B des Periodensystems; und
worin a im Bereich von etwa 0,1 bis etwa 0,9 liegt; und
worin N mindestens ein Metall ist, ausgewählt aus den Metallen in den Gruppen III-A, IV-A, V-A und VI-A des Periodensystems; und
Y ausgewählt ist aus den Gruppen VIII, I-A und II-A des Periodensystems; und
worin b im Bereich von etwa 0,2 bis etwa 0,8 liegt und das die Metalle enthält, die die amorphe Metall-Legierung bilden, unter Bildung der gewünschten amorphen Metall-Legierung, oder unter Bildung eines innigen Gemischs der Komponenten der amorphen Metall-Legierung, das dann einer Wärmebehandlung bei einer Temperatur unter der Kristallisationstemperatur der zu bildenden amorphen Metall-Legierung unterzogen wird, um die amorphe Metall-Legierung zu bilden.

2. Verfahren nach Anspruch 1, dadurch gekennzeichnet, daß die im wesentlichen amorphe Metall-Legierung als ein Pulver erhalten wird.

3. Verfahren nach Anspruch 2, dadurch gekennzeichnet, daß das Pulver weiter zu einer festen Form verarbeitet wird.

4. Verfahren nach einem der Ansprüche 1 bis 3, dadurch gekennzeichnet, daß das innige Gemisch der Komponenten der herzustellenden amorphen Metall-Legierung zu einer Form gepreßt wird.

5. Verfahren nach einem der Ansprüche 1 bis 4, dadurch gekennzeichnet, daß die thermische Zersetzung unter einer inerten Atmosphäre erfolgt.

6. Verfahren nach einem der Ansprüche 1 bis 4, dadurch gekennzeichnet, daß die Zersetzung unter einer reaktiven Atmosphäre erfolgt.

7. Verfahren nach einem der Ansprüche 1 bis 6, dadurch gekennzeichnet, daß eine Zusammensetzung einer amorphen Metall-Legierung hergestellt wird, die nicht-metallischen Elemente einschließt.

8. Verfahren nach Anspruch 7, dadurch gekennzeichnet, daß die Wärmebehandlung des innigen Gemischs unter einer Atmosphäre erfolgt, die die nicht-metallischen Elemente enthält.

9. Verfahren nach einem der Ansprüche 1 bis 8, dadurch gekennzeichnet, daß die Wärmebehandlung des innigen Gemischs unter einer inerten Atmosphäre durchgeführt wird.

10. Verfahren nach einem der Ansprüche 1 bis 9, dadurch gekennzeichnet, daß die Wärmebehandlung des innigen Gemischs unter einer reaktiven Atmosphäre durchgeführt wird.

11. Verfahren nach einem der Ansprüche 1 bis 10, dadurch gekennzeichnet, daß das innige Gemisch Teilchen mit einer maximalen Teilchengröße von 10x10-'° m bis etwa 1000x10⁻¹⁰ m umfaßt.

## Revendications

1. Procédé de synthèse d'un alliage métallique amorphe à au moins 50%, comportant le fait de décomposer thermiquement au moins un composé précurseur contenant un métal, choisi parmi des composés organométalliques tels que des monomères, des dimères, des trimères et des polymères présentant des ligands métallo-organiques composés d'hydrocarbures saturés et/ou insaturés, des ligands aromatiques ou hétéro- aromatiques, ou des ligands content de l'oxygène, du bore, du carbone, de l'azote, du phosphore, de l'arsenic, du germanium, de l'antimoine et/ou du silicium; des composés halogénés; des oxydes; des nitrates; des nitrures; des carbures; des carbonyles; des borures ou des sels contenant un métal, à une température inférieure à la température de cristallisation de l'alliage métallique amorphe à former, le composé précurseur, dont il y a au moins un et qui contient un métal, ayant une température de décomposition inférieure à la température de cristallisation de l'alliage amorphe à former, pour former un produit, résultant de la décomposition, avant les formules . empiriques suivantes:
où M est au moins un métal choisi parmi les métaux des groupes VI-A, VII-A, VIII, IA, IIA et IIIA du tableau périodique; et
X est au moins un élément choisi parmi les groupes III-B, IV-B et V-B du tableau périodique; et
où a est compris entre environ 0,1 et 0,9; et
où N est au moins un métal choisi parmi les métaux des groupes III-A, IV-A, V-A et VI-A du tableau périodique; et
Y est choisi parmi les groupes VIII, I-A et II-A du tableau périodique; et
où b est compris entre environ 0,2 et 0,8; et contenant les métaux qui constituent l'alliage métallique amorphe pour former l'alliage métallique désiré ou pour former un mélange intime des composants de l'alliage métallique amorphe que l'on traite alors thermiquement à une température inférieure à la température de cristallisation de l'alliage métallique amorphe à former, pour former l'alliage métallique amorphe.

2. Procédé selon la revendication 1, caractérisé en ce que l'alliage métallique substantiellement amorphe est obtenu sous forme de poudre.

3. Procédé selon la revendication 2, caractérisé en ce que l'on poursuit le traitement de la poudre pour obtenir une pièce de forme, solide.

4. Procédé selon l'une quelconque des revendications 1 à 3, caractérisé en ce que l'on presse, pour obtenir une pièce de forme, le mélange intime des composants de l'alliage métallique amorphe à synthétiser.

5. Procédé selon l'une quelconque des revendications 1-4, caractérisé en ce que la décomposition thermique se produit sous atmosphère inerte.

6. Procédé selon l'une quelconque des revendications 1 à 4, caractérisé en ce que la décomposition se produit sous atmosphère réactive.

7. Procédé selon l'une quelconque des revendications 1 à 6, caractérisé en ce qu'il synthétise une composition d'alliage métallique amorphe comprenant des éléments non métalliques.

8. Procédé selon la revendication 7, caractérisé en ce que le traitement thermique du mélange intime se fait sous une atmosphère contenant lesdits éléments non-métalliques.

9. Procédé selon l'une quelconque des revendications 1 à 8, caractérisé en ce que le traitement thermique du mélange intime se fait sous atmosphère inerte.

10. Procédé selon l'une quelconque des revendications 1 à 9, caractérisé en ce que ledit traitement thermique du mélange intime se fait sous atmosphère réactive.

11. Procédé selon l'une quelconque des revendications 1 à 10, caractérisé en ce que ledit mélange intime est constitué de particules d'une dimension maximale de particules allant de 10x10-'° m à environ 1000x10-¹⁰ m.
